

## UNITED STATES PATENT OFFICE

2,027,582

## AQUEOUS DISPERSION

Jacob Mitchell Fain, Brooklyn, N. Y., assignor, by  
mesne assignments, to The Patent and Licens-  
ing Corporation, New York, N. Y., a corporation  
of Massachusetts

No Drawing. Original application November 21,  
1928, Serial No. 321,045. Divided and this ap-  
plication January 24, 1931, Serial No. 511,108

15 Claims. (Cl. 134—1)

This is a division of my co-pending application  
Ser. No. 321,045, filed November 21st, 1928.

This invention relates to the art of making  
aqueous dispersions of bituminous and like sub-  
stances normally immiscible with water. Bitu-  
minous dispersions as known to the art at the  
present time, may be produced by various proc-  
esses and with the aid of numerous substances  
functioning as dispersing media to assist in caus-  
ing subdivision of the bitumen into dispersed  
10 particles of more or less fine size. Generally  
speaking, dispersion may be effected by at least  
two distinct types of operations. In one type,  
the dispersing medium functions to reduce the  
15 surface tension of the aqueous medium, this  
being generally evidenced by its ability to foam  
so that dispersion takes place largely by virtue  
of this property, this type of operation being  
normally operable within considerable temper-  
20 ature latitudes within which the phases are  
liquid. Under these conditions, only relatively  
slight mechanical action is necessary to produce  
the dispersion and generally, no great difficulty  
is experienced in attaining fine particle size.  
25 Soap and soapy materials are among the sub-  
stances which function in the foregoing manner  
to produce dispersion, although, of course, other  
materials capable of reducing surface tension of  
the aqueous medium may be utilized.  
30 The dispersion products produced under the  
foregoing conditions and with the aid of the  
aforenamed emulsifying media are frequently  
unstable, and particularly when the amount of  
emulsifying media employed approximates the  
35 minimum that will effect a material reduction in  
the surface tension, the product is unable to  
maintain the dispersed state upon standing for  
substantial periods of time and hence breaks  
down upon standing. With quantities of the  
40 dispersing media in excess of the critical mini-  
mum referred to, the product may be made to  
maintain its dispersed state for substantial  
periods of time although, of course, even in such  
case the introduction of electrolytes and similar  
45 influences, are generally sufficient to cause a  
breaking of the dispersion.

In the other type of operation, the emulsifiers  
employed operate under conditions influenced  
largely by the temperature and the viscosity of  
50 the aqueous dispersion medium. This type of  
operation requires carefully controlled temper-  
atures and considerable internal friction in the  
mass undergoing dispersion with consequent  
aqueous medium in the production of disper-  
55 sions of desirable character. In general, paste

forming powders such as finely divided clays,  
bentonite and the like, are examples of dispers-  
ing media employed in conjunction with this  
second type of operation. When these materials  
are thus employed to produce fine sub-division  
5 of the dispersed particles, the resultant product  
will be comparatively stable, not only in its  
ability to maintain the dispersed state upon  
standing for considerable periods of time, but  
also to the action of most electrolytes.

The object of the present invention is to  
utilize the advantages incident to the type of  
operation first above described for the produc-  
15 tion of dispersions which in certain respects,  
possess the stability characteristic of the prod-  
ucts formed under the second type of operating  
conditions as above described.

Another object of the invention resides in the  
provision of a method for utilizing materials  
capable of reducing the surface tension of the  
20 aqueous medium in the production of dispersions,  
the amount of surface tension reducing  
material employed being regulated to the mini-  
mum necessary to provide, in conjunction with  
materials falling under the second group, a suffi-  
25 cient reduction in surface tension to enable the  
combined media to disperse bitumen in a man-  
ner characteristic of the first type of operation  
above described, yet having far greater stability  
30 (so far as maintaining the dispersed state is  
concerned) than is normally possible with such  
type of operation, the resultant product more  
nearly resembling in this respect the product  
produced with far greater quantity of emulsify-  
35 ing agent of the first type of the product made  
in accordance with the second type of operation.

Other objects of the invention will hereinafter  
more fully appear from the following description  
of the invention.

In carrying out my invention, I may combine  
40 with bentonite and/or clay or other colloidal  
powders capable of forming a paste or viscous  
suspension with water, an agent capable of low-  
ering the surface tension of the aqueous medium  
so as to render the bitumen more readily sus-  
ceptible to rapid subdivision into fine particles  
45 by a comparatively light stirring or agitating  
action. By thus utilizing an agent for reduc-  
ing the surface tension of the asphalt, I am  
enabled to produce dispersions without requir-  
50 ing a very nice and skilled control of the tem-  
perature conditions during the operation, and  
at the same time producing a relatively stable  
product due to the presence therein of the clay,  
55 bentonite or other mineral powder, and without

which the product would be comparatively unstable.

In one embodiment of my invention, I have dispersed a relatively soft asphalt of Columbian stock, the asphalt having a melting point of say between 70 and 90 degrees F., by combining about eight parts of bentonite with one part of soap (sodium oleate) in a solution of about 400 parts of water and dispersing therein approximately 1200 parts by weight of the asphalt, the asphalt in hot molten state being added to the bentonite-soap suspension accompanied by a stirring action performed in any suitable equipment designed for the purpose. The final dispersion as thus produced, as will be seen from the figures given, contains approximately 75% of the asphalt, 25% of water, 0.5% bentonite and  $\frac{1}{8}$ % of soap, each based on the weight of the finished dispersion. These amounts of bentonite and soap total to 0.5625% based on the weight of the dispersion, or 0.75% based on the weight of the asphalt. With such a small proportion of the soap, this product, in the absence of the bentonite, would normally be comparatively unstable and in fact, breaks down upon standing for any considerable length of time, say a few weeks. Due to the presence of the bentonite, however, this disruption of the product is prevented. On the other hand, it will be apparent to those skilled in the art, that in order to satisfactorily disperse asphalt of such a soft nature with a small amount of material like bentonite, a very careful control of the temperature conditions during the operation would be necessary, but that, in accordance with my invention, the necessity for this control is eliminated due to the function of the soap, the operation thus resembling the dispersion of asphalt with materials like soap, in that the same may be carried on at relatively high temperatures varying over a considerable range, which would ordinarily seriously encumber the operation when using material such as bentonite or the like.

In another embodiment of my invention I may use saponin as the surface tension reducing material in lieu of soap. To produce dispersion with this material I may combine the same with a paste forming colloid such as bentonite in proportions say of one part of the saponin to say one to about three parts of bentonite. With these proportions I may produce a stable dispersion of asphalt of the above described character and containing about 70 to 75% of the asphalt, 30 to 25% of water, about  $\frac{1}{4}$ % saponin, and  $\frac{1}{4}$ % to  $\frac{3}{4}$ % bentonite. Here again the combined weight of saponin and bentonite is not more than 1% by weight of the finished dispersion and also less than 2% by weight of the asphalt contained in the dispersion.

I may also carry out my invention by combining soap with an aqueous mixture of gelatin in quantities to reduce sufficiently the surface tension of the aqueous medium so as to enable satisfactory dispersion to take place. With this procedure and using approximately two parts of gelatin to each part of soap, the final dispersion may contain approximately 70 to 75% of the bitumen, about  $\frac{1}{4}$ % soap,  $\frac{1}{2}$ % gelatin, and the balance water, i. e., about  $\frac{3}{4}$ % of soap and gelatin combined, based on the weight of the dispersion, or about 1% of soap and gelatin combined, based on the weight of the bitumen contained in the dispersion.

The last named procedure may also be car-

ried out with the substitution of saponin in lieu of the soap, in which event the dispersion produced may contain about  $\frac{3}{4}$ % saponin,  $\frac{1}{2}$ % gelatin, the bitumen and water content being approximately the same as that stated. The final product in such case would therefore contain 1.25% of saponin and gelatin combined, based on the weight of the dispersion, or 1.66% based on the weight of the bitumen contained in the dispersion.

It should be understood that in the illustrations hereinabove given, the stability of the product may be even further increased within certain limits, by increasing the relative amount of the bentonite or similar substance present in the dispersion, this regulation of the stability of the final product, obviously depending upon the degree of stability desired for the particular use to which it is to be applied.

The present invention produces a product ordinarily requiring a rather accurate control by a process eliminating the requirement for such control.

I claim as my invention:

1. An aqueous dispersion of bitumen comprising not substantially less than 50% by weight of bitumen and containing a mixture of soluble soap and a mineral powder colloid as the primary emulsifying agent and not less than 25% of water as the continuous phase, said soap and mineral powder colloid being present in a combined amount less than 1% by weight of the dispersion.

2. An aqueous dispersion of bitumen comprising not substantially less than 50% by weight of bitumen and containing a mixture of soluble soap and a mineral powder colloid as the primary emulsifying agent and not less than 25% of water as the continuous phase, said soap and mineral powder colloid being present in a combined amount less than 1% by weight of the bitumen contained in the dispersion.

3. An aqueous dispersion of bitumen comprising not substantially less than 50% by weight of bitumen and containing a mixture of soluble soap and bentonite as the primary emulsifying agent and not less than 25% of water as the continuous phase, said soap and bentonite being present in a combined amount less than 1% by weight of the dispersion.

4. An aqueous dispersion of bitumen comprising not substantially less than 50% by weight of bitumen and containing a mixture of soluble soap and bentonite as the primary emulsifying agent and not less than 25% of water as the continuous phase, said soap and bentonite being present in a combined amount less than 1% by weight of the bitumen contained in the dispersion.

5. An aqueous dispersion of bitumen comprising not substantially less than 50% by weight of bitumen and containing a mixture of soluble soap and a mineral powder colloid as a primary emulsifying agent and not less than 25% of water as the continuous phase, said soap being present in an amount less than 1% by weight of the dispersion and said mineral powder colloid being present in an amount less than 1% by weight of the bitumen contained in the dispersion.

6. An aqueous dispersion of bitumen comprising not substantially less than 50% by weight of bitumen and containing a mixture of soluble soap and a mineral powder colloid as the primary emulsifying agent and not less than 25% 75

of water as the continuous phase, said soap being present in an amount less than 1% by weight of the bitumen contained in the dispersion, and said mineral powder colloid being present in an amount less than 1% by weight of the dispersion.

7. An aqueous dispersion of bitumen comprising not substantially less than 50% by weight of bitumen and containing a mixture of soluble soap and bentonite as the primary emulsifying agent and not less than 25% of water as the continuous phase, said soap being present in an amount less than 1% by weight of the dispersion and said bentonite being present in an amount less than 1% by weight of the bitumen contained in the dispersion.

8. An aqueous dispersion of bitumen comprising not substantially less than 50% by weight of bitumen and containing a mixture of soluble soap and bentonite as the primary emulsifying agent and not less than 25% of water as the continuous phase, said soap being present in an amount less than 1% by weight of the bitumen contained in the dispersion, and said bentonite being present in an amount less than 1% by weight of the dispersion.

9. An aqueous dispersion of bitumen comprising not substantially less than 50% by weight of bitumen and containing a mixture of soluble soap and a mineral powder colloid as the primary emulsifying agent and not less than 25% of water as the continuous phase, said soap and colloid being present in a combined amount less than 2% by weight of the dispersion.

10. An aqueous dispersion of bitumen comprising not substantially less than 50% by weight of bitumen and containing a mixture of soluble soap and bentonite as the primary emulsifying agent and not less than 25% of water as the continuous phase, said soap and bentonite being present in a combined amount less than 2% by weight of the dispersion.

11. An aqueous dispersion of bitumen comprising not substantially less than 50% by weight of bitumen and containing not less than 25% by weight of water and containing as the primary emulsifying agent a mixture of less than 1% soap and less than 1% bentonite, both based on the weight of the dispersion.

12. An aqueous dispersion of bitumen comprising not substantially less than 50% by weight of bitumen and containing not less than 25% by weight of water and containing as the primary emulsifying agent a mixture of less than  $\frac{1}{2}\%$  soap and not more than  $\frac{1}{2}\%$  bentonite, both based on the weight of the dispersion.

13. An aqueous dispersion of bitumen comprising not substantially less than 50% by weight of bitumen and containing not less than 25% by weight of water and containing as the primary emulsifying agent a mixture of less than 1% soap and not more than 1% bentonite, both based on the weight of the dispersion.

14. An aqueous dispersion of bitumen comprising not substantially less than 50% by weight of bitumen and containing not less than 25% by weight of water and containing as the primary emulsifying agent a mixture of soluble soap in an amount less than 1% by weight of the dispersion and bentonite in an amount less than 1% by weight of the dispersion, but sufficient to maintain the uniformly dispersed state of the product upon standing over considerable periods of time.

15. An aqueous dispersion of bitumen comprising not substantially less than 50% by weight of bitumen, not less than 25% by weight of water, and a combination of soap and bentonite as the primary emulsifying agent in an amount not exceeding 2% by weight of the bitumen contained in the dispersion.

40

JACOB MITCHELL FAIN.